

# UNITED STATES PATENT OFFICE.

HARRY ORMISTON ORMISTON, OF ROCKDALE, NEAR SYDNEY, NEW SOUTH WALES,  
AUSTRALIA.

## METALLIC ALLOY AND PROCESS OF MANUFACTURE THEREOF.

1,101,089.

Specification of Letters Patent. Patented June 23, 1914.

No Drawing.

Application filed February 11, 1913. Serial No. 747,726.

To all whom it may concern:

Be it known that I, HARRY ORMISTON ORMISTON, subject of the King of Great Britain and Ireland, residing at Chapel 5 street, Rockdale, near Sydney, in the State of New South Wales, Australia, have invented a certain new and useful Improved Metallic Alloy and Process of Manufacture Thereof, of which the following is a specification.

My invention relates to production of metallic alloys of the class in which the chief constituent is aluminium, and it comprises an alloy metal or stock metal containing 15 aluminium, nickel, copper, cadmium, tin, and lead, which metals are intermixed and associated by a particular process. Said metallic alloy is bright and white in color and exhibits valuable properties some of 20 which distinguish it from its chief constituent, aluminium viz. it may be brazed, soldered, turned, rolled, drawn, or forged, or welded by means of the oxyacetylene jet; it may be varied in hardness and tensile 25 strength; it takes a high polish; and it is highly resistant to oxidation by atmospheric and weather influences. In manufacturing said alloy it is necessary to proceed in stages. In the first stage I fuse in a crucible, certain 30 salts of sodium, magnesium, copper, mercury, cadmium and nickel; in the second stage I add metallic nickel and copper to the fused salts, which latter act as a flux as well as having the functions of adding metallic elements to the final product, and 35 maintain the temperature till the body of the mass is in a quiet fluid condition and intermixed; and then I introduce gradually metallic tin, lead, and aluminium into the 40 crucible containing the before mentioned substances, and maintain the temperature until complete fusion and thorough incorporation of metals is effected, stirring the fused mass to facilitate separation of metal 45 from dross. The fused product thus obtained is a stock alloy with which further aluminium, tin, lead, copper and nickel may be subsequently alloyed to produce commercial alloys of different kinds.

50 The approximate proportions of the components hereinafter set forth should be used to obtain the most beneficial results. No substantial variation is permissible without more or less modifying the desired characteristics of the final alloy, except in the case

of the magnesium sulfate. The chief effect of magnesium sulfate is to brighten the color of the metal; and it may be entirely omitted without material prejudice to the qualities (other than color) of the metal.

In the first stage of the manufacture, I advantageously take my materials in the following proportions by weight: borax 60 parts, magnesium sulfate 5 parts, copper sulfate 10 parts, copper nitrate 7 parts, mercuric sulfate 1 part, cadmium sulfate 2 parts, and nickel sulfate 15 parts, or a total of 100 parts by weight. Sodium bicarbonate may be substituted for borax, though borax is preferred as it makes a better flux and slag. 70 Copper sulfate or copper nitrate may be used, or copper sulfate and copper nitrate. The proportions of sodium and copper in the abovementioned relative quantities of the salts thereof should be maintained approximately. This mixture which I term the "flux" is placed in a crucible and the temperature raised. While the ebullition is active I add to the stated amount of material approximately 3 parts of metallic nickel and 80 3 parts of metallic copper, and maintain the temperature until ebullition has ceased or almost ceased. I then add 3 parts of metallic tin, one part of metallic lead, and 90 parts of metallic aluminium. It is desirable 85 to add the aluminium gradually rather than to introduce it into the crucible in mass as its reductive action is apt to be too energetic. The contents of the crucible are finally stirred with an iron rod to facilitate 90 separation of metal from dross or slag before the metal is poured. There will collect around the top of the crucible a ring of borax and products of the other materials which served as flux; this slag or dross is 95 readily removed, and the alloy is left in a very fluid condition which it maintains as long as the temperature is maintained. It may be cast at once and remelted as often as required without affecting its characteristic qualities. The alloy so produced forms a 100 stock metal which may be remelted and used to form commercial alloys having different characteristics. To obtain soft and ductile alloys it is remelted with aluminium in a 105 wide range of proportions, varying up to 90% of aluminium in the total weight; in this case one part of metallic tin and one fourth part of metallic lead are preferably also added for every twenty parts of addi- 110

- tional aluminium which is to be alloyed with the stock metal, the additions being made gradually. I have used mixtures containing 20 parts stock metal, 9 parts tin, 2 parts lead, and 169 parts aluminium, and have found this product preferable to a product containing additional aluminium only. To obtain hard metal, the stock metal is remelted with aluminium and copper, a very hard product being obtained by alloying 20 parts copper and 50 parts aluminium with 30 parts of the stock, and products of lesser hardness with alloys containing a smaller proportion of copper. Another hard metal may be made by introducing into the 100 parts of "flux" beforementioned during ebullition (instead of the quantities previously stated) 30 parts metallic nickel, and 5 parts of metallic copper which metals are added gradually and when the ebullition has subsided adding 57 parts metallic aluminium, 6 parts metallic tin, and 2 parts metallic lead. A solder usable for uniting any of these metals together or to other metals is made by alloying one of the final alloys above described with tinman's solder (lead 66 per cent. and tin 34 per cent. approximately) in the proportion of two to one, which proportion admits of considerable variation. In making a solder joint no flux need be used with my metal in joining it together or in joining it to aluminium but the usual fluxes may be used with copper, iron and other metals.
- The special solder above described is used to "tin" the surfaces to be united, and then ordinary tinman's solder may be used to make the joint.
- What I claim as my invention and desire to secure by Letters Patent is:
1. A stock alloy comprising aluminium, nickel, copper, tin, cadmium and lead.
  2. The process of making useful alloys which comprises melting a copper salt, a cadmium salt, a nickel salt, a mercury salt and a fluxing sodium salt together and adding metal comprising aluminium.
  3. The process of making useful alloys which comprises melting a copper salt, a cadmium salt, a nickel salt, a mercury salt, 50 a magnesium salt and a fluxing sodium salt together and adding metal comprising aluminium.
  4. The process of making useful alloys which comprises melting copper sulfate and nitrate, cadmium sulfate, mercuric sulfate, nickel sulfate and a fluxing sodium salt together and adding metal comprising aluminium.
  5. The process of making useful alloys which comprises melting copper sulfate and nitrate, cadmium sulfate, mercuric sulfate, nickel sulfate, magnesium sulfate and a fluxing sodium salt together and adding metal comprising aluminium.
  6. The process of making useful alloys which comprises melting a copper salt, a cadmium salt, a nickel salt, a mercury salt and a fluxing sodium salt together, while ebullition is active adding nickel and copper, 70 maintaining hot until ebullition practically ceases, and adding tin, lead and aluminium.
  7. The process of making useful alloys which comprises melting copper sulfate, copper nitrate, mercury sulfate, cadmium sulfate, nickel sulfate and a fluxing sodium salt together, while ebullition is active adding nickel and copper, maintaining hot until ebullition practically ceases, and adding tin, lead and aluminium.
  8. The process of making useful alloys which comprises melting 5 parts magnesium sulfate, 10 parts copper sulfate, 7 parts copper nitrate, 1 part mercury sulfate, 2 parts cadmium sulfate, 15 parts nickel sulfate and 60 parts borax together, while the mixture is still in active ebullition adding 3 parts metallic nickel and 3 parts metallic copper, and after ebullition practically ceases adding 3 parts tin, 1 part lead and 90 parts metallic 80 aluminium.

In testimony whereof I have affixed my signature in presence of two witnesses.

HARRY ORMISTON ORMISTON.

Witnesses:

W. J. DAVIS,  
H. H. RITCHING.